

1

3,161,513

**PHOTOGRAPHIC DEVELOPER COMPOSITIONS  
CONTAINING AN ANTISTAIN AGENT**

Richard W. Henn, Rochester, N.Y., assignor to Eastman Kodak Company, Rochester, N.Y., a corporation of New Jersey  
No Drawing. Filed Mar. 22, 1961, Ser. No. 97,421  
8 Claims. (Cl. 96—61)

This invention relates to photographic developer compositions and more particularly to nonstaining photographic developer compositions for black and white photographic emulsions.

When silver halide negative emulsions are developed under conditions having considerable solvent action for the silver halide a silver stain or scum tends to be formed. This is particularly so when high speed silver halide negative emulsions are developed in fine grain photographic developers which exert considerable solvent action for the silver halide. The stain is usually metallic by reflected light, and yellow or brown by transmitted light, and may have considerable printing density.

While high speed negative silver halide emulsions are most subject to staining nearly all silver halide emulsions may develop a scum or stain when developed in a developer solution having considerable solvent action for the silver halide. Thus, high speed black-and-white silver halide printing papers tend to stain when developed in a developer solution containing sufficient solvent for the silver halide. Accordingly, the utility of the nonstaining photographic developer compositions of the invention is not restricted to the development of high speed negative silver halide emulsions.

The silver stain or scum, usually referred to herein simply as stain, is more likely to be produced in used photographic developer solutions than in fresh photographic developer solutions and becomes increasingly pronounced with extended developing times. Further, aged silver halide negative photographic films have a greater tendency to produce silver stain than the corresponding fresh silver halide negative photographic films.

It is an object of this invention to prevent the formation of stain when silver halide emulsions are developed. A particular object is to prevent the formation of stain when silver halide negative emulsions are developed. A further object is to provide photographic developer compositions containing an agent which prevents or greatly reduces staining. Another object is to provide fine grain photographic developer compositions of improved properties. A further object is to provide a process for developing silver halide emulsions, especially silver halide negative emulsions, under conditions having considerable solvent action for silver halide, in the presence of an agent which effectively inhibits staining.

I have discovered that 2,4-dihydroxybenzophenone effectively inhibits the formation of the stain or scum which is frequently produced when high speed silver halide negative emulsions are developed under conditions having considerable solvent action for the silver halide. Thus, 2,4-dihydroxybenzophenone inhibits or prevents the formation of the stain or scum which is ordinarily produced when high speed silver halide negative emulsions are developed in fine grain photographic developer solutions which exert considerable solvent action for the silver halide. The 2,4-dihydroxybenzophenone is normally added to the developer composition. However, it may be incorporated in the photographic emulsion. As the developer solution becomes exhausted it can be renewed by the addition of a developer-replenisher solution containing a suitable amount of 2,4-dihydroxybenzophenone.

As indicated hereinbefore, 2,4-dihydroxybenzophenone also effectively inhibits the formation of the stain or scum

2

that tends to be formed when high speed black-and-white silver halide printing papers are developed in a developer solution having considerable solvent action for the silver halide. While 2,4-dihydroxybenzophenone is of most utility when used in connection with the development of silver halide emulsions which are most likely to produce stain or scum it can be usefully employed in the development of any silver halide emulsion which tends to produce stain or scum.

10 The amount of 2,4-dihydroxybenzophenone used varies from about 0.02 to about 5.0 grams per liter of developing solution. The preferred range is from about 0.1 to about 1.0 gram per liter of developing solution. The addition of even the lowest concentration of 2,4-dihydroxybenzophenone materially reduces the intensity of the stain. Higher concentrations frequently entirely prevent staining.

15 2,4-dihydroxybenzophenone has powerful antistain action, has suitable physical properties, may be employed in low concentrations and has little sensitometric effect.

20 Illustrative of the silver halide negative emulsions that can be advantageously developed in the presence of 2,4-dihydroxybenzophenone are the emulsions present in Kodak Panatomic-X, Kodak Verichrome Pan, Kodak Plus-X Pan, Kodak Tri-X Pan, Kodak Royal-X Pan, Ansco All-Weather Pan, Ansco Super Hypan, Ansco Superpan Press, Gevaert X-L Pan, Ilford HP-3, Ilford HP-S and Ilford FP-3 photographic film. All of these photographic films have negative speed silver bromoiodide emulsions. They are merely illustrative and not limitative of the photographic films that can be developed with advantage in the presence of 2,4-dihydroxybenzophenone.

25 Printing papers containing high speed silver bromoiodide emulsions are illustrative of the printing papers that can be developed with advantage in the presence of 2,4-dihydroxybenzophenone.

30 The photographic films mentioned hereinbefore and other brands of photographic film corresponding thereto, have high speed silver halide negative emulsions even though the various emulsions vary greatly in their speed ratings.

35 The use of 2,4-dihydroxybenzophenone as an antistain agent is not restricted to any particular photographic developer or class of photographic developers. So far as I am aware it can be used with any of the known photographic developers. The photographic developer solution can have the agents usually present therein, e.g. photographic developer, a preservative such as sodium sulfite and an alkaline agent such as sodium hydroxide or sodium carbonate. Other ingredients such as potassium bromide, benzotriazole or toners, for example, can also be present. Hydroquinone, paramethylaminophenol sulfate, paraphenylenediamine, p-aminophenol, 1-phenyl-3-pyrazolidone, 4,4-dimethyl-1-phenyl-3-pyrazolidone, 1-phenyl-4-ethyl-3-pyrazolidone, 2,4-diaminophenol and pyrogallol are illustrative of the developing agents that can be employed. Mixtures of developing agents such as hydroquinone and paramethylaminophenol sulfate, and 4,4-dimethyl-1-phenyl-3-pyrazolidone and hydroquinone, for example, can be employed.

40 Sodium thiocyanate, potassium thiocyanate, ammonium thiocyanate, sodium chloride, ammonium chloride, ethylene diamine, 1,3,5-triaminobenzene, ethanolamine, diethanolamine, sodium thiosulfate and sodium sulfite are illustrative of the silver halide solvents that can be present during the development step.

45 The following examples illustrate my invention.

**EXAMPLE 1**

50 Strips of Kodak Royal-X Pan Film which had been incubated for one week at 120° F. were tested in Kodak Developer DK-50 and in this developer having varying amounts of 2,4-dihydroxybenzophenone (0.1 and 0.5

gram per liter) therein. These developer solutions are referred to as 1, 2 and 3 for purpose of reference. The strips were developed in large test tubes of developer solution at 68° F. for 10 minutes. As each strip was removed from the developer solution a portion of the strip was wiped with the fingers in order that the stained area could be more readily detected and compared with a clear area. The strips were then immersed in a stop bath, fixed, and washed with water. The developer solution containing no 2,4-dihydroxybenzophenone produced an intense stain whereas the developer solutions containing 2,4-dihydroxy benzophenone produced little or no stain.

The results obtained are tabulated hereinafter.

| Developer: | Stain density |
|------------|---------------|
| 1          | 0.06          |
| 2          | 0.01          |
| 3          | 0.00          |

#### EXAMPLE 2

A solution of Kodak Developer DK-50 containing 0.2 gram of 2,4-dihydroxybenzophenone per liter of developer solution was exhausted by the processing of successive rolls of Kodak Verichrome Pan Film having 80 square inches of emulsion per roll. After each roll of film was developed 11 cc. of Kodak Replenisher DK-50R solution, modified by the addition of 0.5 gram of 2,4-dihydroxybenzophenone per liter of solution, were added to the developer solution. No stain was encountered at any stage of the processing, even after developing the equivalent of 400 rolls per gallon of the starting developer solution. By contrast, the unmodified Kodak Developer DK-50 and unmodified Kodak Replenisher DK-50R used as a control produced high dichroic silver stain.

Kodak Developer DK-50 and Kodak Replenisher DK-50R, and their use, are described, for example, in the Kodak Data Book, 5th edition (first 1960 printing), entitled "Processing Chemicals and Formulas for Black-and-White Photography".

The 2,4-dihydroxybenzophenone antistaining or anti-scumming agent of my invention can be added to combined developing and fixing compositions and to combined developing and stabilizing compositions. Thus, 2,4-dihydroxybenzophenone may be added to the monobath compositions disclosed, for example, in Haist et al. U.S. Patent 2,875,048, issued February 24, 1959, Dreywood U.S. Patent 2,525,532, issued October 10, 1959, King U.S. Patent 2,397,016, issued March 19, 1946, Goldhammer et al. U.S. Patent 2,782,120, issued February 19, 1957, and Goldhammer U.S. Patents 2,782,121 and 2,901,350, issued February 19, 1957, and August 25, 1959, respectively. Some of these combined developer and fixer or developer and stabilizer compositions can be prepared in dry form for making working solutions.

Kodak Developer DK-50 contains the following ingredients per liter of solution.

|                               | Grams |
|-------------------------------|-------|
| Paramethylaminophenol sulfate | 2.5   |
| Sodium sulfite, desiccated    | 30.0  |
| Hydroquinone                  | 2.5   |
| Sodium bisulfite              | 15.0  |
| Sodium metaborate             | 10.0  |
| Potassium bromide             | 0.5   |

As indicated hereinbefore, this developer composition can be modified by the addition of about 0.002 to about 5.0 grams of 2,4-dihydroxybenzophenone. Preferably, about 0.1 to about 1.0 gram of 2,4-dihydroxybenzophenone is added. Representative developer compositions are obtained, for example, by the addition of 0.1 gram, 0.2 gram, 0.5 gram, 1.0 gram and 2.0 grams, respectively, of 2,4-dihydroxybenzophenone to the above composition, although smaller and larger amounts may be added.

Other photographic developers that can be modified with 2,4-dihydroxybenzophenone include Kodak Developer D-23, Kodak Developer D-25, Kodak Developer D-76, Kodak Developer SD-21 and Kodak Developer SD-28, for example. These developers are merely illustrative and not limitative of the developers that can be modified with 2,4-dihydroxybenzophenone.

The 2,4-dihydroxybenzophenone antistaining agent of my invention may be incorporated in stable, dry, single powder photographic developer compositions of the types described, for example, by Kridel et al. U.S. Patents 2,666,702 and 2,666,703, issued January 19, 1954, Wiitala et al. U.S. Patents 2,682,464 and 2,682,465, issued June 29, 1954, Henn et al. U.S. Patent 2,685,513, issued August 3, 1954, and Baxendale et al. U.S. Patent 2,816,026, issued December 10, 1957.

Representative stable, dry, single powder photographic developer compositions containing 2,4-dihydroxybenzophenone are set forth hereinafter.

#### EXAMPLE 3

|                              | Grams |
|------------------------------|-------|
| Elon                         | 2.0   |
| Hydroquinone                 | 8.0   |
| Sodium sulfite (desiccated)  | 90.0  |
| Sodium carbonate monohydrate | 52.5  |
| Potassium bromide            | 5.0   |
| Boric anhydride              | 1.6   |
| Phthalic anhydride           | 0.16  |
| 2,4-dihydroxybenzophenone    | 1.0   |

#### EXAMPLE 4

|                                          |      |
|------------------------------------------|------|
| Elon                                     | 2.5  |
| Sodium sulfite (desiccated)              | 30.0 |
| Hydroquinone                             | 2.5  |
| Sodium metaborate (10% H <sub>2</sub> O) | 10.5 |
| Potassium bromide                        | 0.5  |
| Boric anhydride                          | 0.5  |
| Phthalic anhydride                       | 0.05 |
| 2,4-dihydroxybenzophenone                | 0.5  |

#### EXAMPLE 5

|                              |      |
|------------------------------|------|
| Elon                         | 2.2  |
| Anhydrous sodium sulfite     | 96.0 |
| Hydroquinone                 | 8.8  |
| Sodium carbonate monohydrate | 57.5 |
| Potassium bromide            | 5.0  |
| Metaboric acid               | 3.4  |
| 2,4-dihydroxybenzophenone    | 0.1  |

#### EXAMPLE 6

|                                          |      |
|------------------------------------------|------|
| Elon                                     | 2.5  |
| Anhydrous sodium sulfite                 | 30.0 |
| Hydroquinone                             | 2.5  |
| Sodium metaborate (10% H <sub>2</sub> O) | 10.5 |
| Potassium bromide                        | 0.5  |
| Metaboric acid                           | 4.7  |
| 2,4-dihydroxybenzophenone                | 0.5  |

#### EXAMPLE 7

|                              |      |
|------------------------------|------|
| Elon                         | 3.0  |
| Sodium sulfite               | 45.0 |
| Hydroquinone                 | 12.0 |
| Sodium carbonate monohydrate | 80.0 |
| Potassium bromide            | 0.6  |
| 5-methyl benzotriazole       | 0.06 |
| Metaboric acid               | 1.4  |
| 2,4-dihydroxybenzophenone    | 1.0  |

The foregoing stable, dry, single powder photographic developer compositions are merely illustrative and not limitative.

The compositions for Kodak Developer SD-21 and Kodak Developer SD-28 are given hereinafter.

## Kodak Developer SD-21

|                                              | Grams |
|----------------------------------------------|-------|
| Elon (paramethylaminophenol sulfate)         | 2.0   |
| Hydroquinone                                 | 5.0   |
| Na <sub>2</sub> SO <sub>3</sub> (desiccated) | 100.0 |
| Borax                                        | 8.0   |
| Boric acid                                   | 8.0   |
| KBr                                          | 0.25  |
| H <sub>2</sub> O to make 1 liter.            |       |

## Kodak Developer SD-28

|                                              |      |
|----------------------------------------------|------|
| Elon (paramethylaminophenol sulfate)         | 1.5  |
| Hydroquinone                                 | 1.3  |
| Na <sub>2</sub> SO <sub>3</sub> (desiccated) | 75.0 |
| Borax                                        | 4.5  |
| KBr                                          | 0.4  |
| H <sub>2</sub> O to make 1 liter.            |      |

The compositions for Kodak Developer D-23, Kodak Developer D-25 and Kodak Developer D-76 are given hereinafter.

## Kodak Developer D-23

|                               |       |       |
|-------------------------------|-------|-------|
| Water, about 125 F. (50 C.)   | cc    | 750   |
| Elon                          | grams | 7.5   |
| Sodium sulfite, desiccated    | do    | 100.0 |
| Cold water to make 1.0 liter. |       |       |

Dissolve chemicals in the order given.

## Kodak Developer D-25

|                               |       |       |
|-------------------------------|-------|-------|
| Water, about 125 F. (50 C.)   | cc    | 750   |
| Elon                          | grams | 7.5   |
| Sodium sulfite, desiccated    | do    | 100.0 |
| Sodium bisulfite              | do    | 15.0  |
| Cold water to make 1.0 liter. |       |       |

Dissolve chemicals in the order given.

## Kodak Developer D-76

|                             |       |       |
|-----------------------------|-------|-------|
| Water, about 125 F. (50 C.) | cc    | 750   |
| Elon                        | grams | 2.0   |
| Sodium sulfite, desiccated  | do    | 100.0 |
| Hydroquinone                | do    | 5.0   |
| Borax, granular             | do    | 2.0   |
| Water to make 1.0 liter.    |       |       |

Dissolve chemicals in the order given.

I have also discovered that m-cresol, ortho phenylphenol, pentachlorophenol and thiobenzanilide possess antistaining activity.

The invention has been described in detail with particular reference to preferred embodiments thereof, but it will be understood that variations and modifications can be effected within the spirit and scope of the invention as described hereinabove and as defined in the appended claims.

I claim:

1. A photographic developing solution containing an organic silver halide photographic developer selected from the group consisting of hydroquinone, paramethylaminophenol sulfate, paraphenylenediamine, p-aminophenol, 2,4-diaminophenol, pyrogallol and a 1-phenyl-3-pyrazolidone, a silver halide solvent in sufficient amount to exert considerable solvent action for silver halide and from about 0.02 to about 5.0 grams of 2,4-dihydroxybenzophenone per liter of the developing solution.

2. A photographic developing solution containing an organic silver halide photographic developer selected from the group consisting of hydroquinone, paramethylaminophenol sulfate, paraphenylenediamine, p-aminophenol, 2,4-diaminophenol, pyrogallol and a 1-phenyl-3-pyrazolidone, a silver halide solvent in sufficient amount to exert considerable solvent action for silver halide and from about 0.1 to about 1.0 gram of 2,4-dihydroxybenzophenone per liter of the developing solution.

3. As a new photographic developer composition, an

aqueous solution comprising an alkaline material, an organic silver halide photographic developer selected from the group consisting of hydroquinone, paramethylaminophenol sulfate, paraphenylenediamine, p-aminophenol, 2,4-diaminophenol, pyrogallol and a 1-phenyl-3-pyrazolidone, sodium sulfite in sufficient amount to exert considerable solvent action for silver halide and from about 0.02 to about 5.0 grams of 2,4-dihydroxybenzophenone per liter of the developer solution.

4. As a new photographic developer composition an aqueous solution comprising paramethylaminophenol sulfate, an alkaline material, sodium sulfite in sufficient amount to exert considerable action for silver halide and from about 0.02 to about 5.0 grams of 2,4-dihydroxybenzophenone per liter of the developer solution.

5. In the process for developing an exposed high speed silver halide emulsion with an organic silver halide photographic developer selected from the group consisting of hydroquinone, paramethylaminophenol sulfate, paraphenylenediamine, p-aminophenol, 2,4-diaminophenol, pyrogallol and a 1-phenyl-3-pyrazolidone, under conditions which exert considerable solvent action for the silver halide the improvement which consists in carrying out the developing reaction in the presence of from about 0.02 to about 5.0 grams of 2,4-dihydroxybenzophenone per liter of the developer solution.

6. In the process for developing an exposed high speed silver halide negative emulsion with an organic silver halide photographic developer selected from the group consisting of hydroquinone, paramethylaminophenol sulfate, paraphenylenediamine, p-aminophenol, 2,4-diaminophenol, pyrogallol and a 1-phenyl-3-pyrazolidone, under conditions which exert considerable solvent action for the silver halide the improvement which consists in carrying out the developing reaction in the presence of from about 0.02 to about 5.0 grams of 2,4-dihydroxybenzophenone per liter of the developer solution.

7. A photographic developer solution containing as its essential ingredients for one liter of developer solution:

|                               | Grams       |
|-------------------------------|-------------|
| Paramethylaminophenol sulfate | 2.5         |
| Sodium sulfite, desiccated    | 30.0        |
| Hydroquinone                  | 2.5         |
| Sodium bisulfite              | 15.0        |
| Sodium metaborate             | 10.0        |
| Potassium bromide             | 0.5         |
| 2,4-dihydroxybenzophenone     | 0.02 to 5.0 |

8. A photographic developer solution containing as its essential ingredients for one liter of developer solution:

|                               | Grams      |
|-------------------------------|------------|
| Paramethylaminophenol sulfate | 2.5        |
| Sodium sulfite, desiccated    | 30.0       |
| Hydroquinone                  | 2.5        |
| Sodium bisulfite              | 15.0       |
| Sodium metaborate             | 10.0       |
| Potassium bromide             | 0.5        |
| 2,4-dihydroxybenzophenone     | 0.1 to 1.0 |

## References Cited in the file of this patent

## UNITED STATES PATENTS

|           |              |               |
|-----------|--------------|---------------|
| 2,279,514 | Ham et al.   | Apr. 14, 1942 |
| 2,682,559 | Stanley      | June 29, 1954 |
| 2,983,604 | Duffy et al. | May 9, 1961   |

## OTHER REFERENCES

Glafkides: "Photographic Chemistry," vol. 1, page 129, Fountain Press, London (1958).

Henn et al.: PSA Journal, vol. 19B, pages 146-8 (1953).

Neblette: Photography, Its Materials and Processes, 5th ed., D. Van Nostrand Co., Inc., New York, 1952, pages 205-208, 213, 214.